

# UNITED STATES PATENT OFFICE.

GEORGE ALBERT CHAPMAN, OF ANACONDA, MONTANA, ASSIGNOR, BY MESNE ASSIGNMENTS, TO MINERALS SEPARATION NORTH AMERICAN CORPORATION.

## ORE CONCENTRATION.

1,234,288.

Specification of Letters Patent.

Patented July 24, 1917.

No Drawing. Application filed September 30, 1914, Serial No. 864,820. Renewed June 20, 1917. Serial No. 175,978.

*To all whom it may concern:*

Be it known that I, GEORGE ALBERT CHAPMAN, a subject of the King of England, residing at Anaconda, Deerlodge county, State 5 of Montana, United States of America, have invented certain new and useful Improvements in Ore Concentration, of which the following is a specification.

This invention is for improvements in or 10 relating to ore concentration and has particular reference to the concentration of ores by flotation, for example by the well-known agitation froth process.

As is well-known the formation of a mineral bearing froth in that process is assisted 15 by the fine pulverization of the ore, or by the presence in the ore pulp of a certain proportion of slime mineral. In the case of certain ores, however, a part of the 20 slimes (both mineral and gangue, or either) is in a colloidal or quasi-colloidal state; and it is found that the presence of colloidal slimes in the pulp, if in excess of that 25 which may be usefully employed in assisting in the formation of good stable froths, is a serious impediment to the successful concentration of the sulfid values in such an ore. In some instances this interference 30 has been to some extent overcome by the dilution of the pulp so as to diminish the proportion of solids in suspension. In other cases the processes as described in the previous United States Patents No. 1,102,873 35 to myself and Tucker and No. 1,102,874 to myself, both issued July 7, 1914, have been successfully applied to ores of this type. In some cases where the proportion of colloids has been very high it has been hitherto difficult or impossible to effect commercial 40 or profitable separation by the flotation treatment of such an ore. The actual cause of failure has not been scientifically explained in detail. Apparently the tendency is for the colloid matter in suspension to 45 adsorb or otherwise render ineffective the frothing agents which are used.

An attempt has been made to employ in admixture with the pulp certain coagulable materials with the object of bringing about 50 a settlement of the suspended matter but it is found that during coagulation and settlement the sulfid mineral particles are collected in the coagulations and cannot thereafter be separated by flotation.

An essential feature of this invention 55 consists in adding to the pulp certain substances containing acid radicals of oxyacids of the aliphatic group which enable an ore pulp containing a large proportion of colloidal particles to be successfully treated 60 by flotation. As these substances have been found effective in dealing with ores containing colloidal gangues I have termed them colloid agents.

The colloid agents which have been found 65 most effective are tartaric acid or citric acid or salts of these such as argol, employed in solution in the pulp.

In practice the pulp of powdered ore and 70 water is prepared as usual and a very small proportion of the colloid agent, such as tartaric acid or argol is added thereto, before or during the agitation and aeration.

This invention may advantageously be used in conjunction with the processes described in the previous United States Patents Nos. 1,102,873 and 1,102,874, above referred to, that is to say, the water to be used in the froth flotation process may be agitated with a modifying agent such as 75 cresol or the like and with the colloid agent, before coming into contact with the ore to be treated: or the ore may be ground with water containing the colloid agent or containing both the colloid agent and a modifying agent such as cresol. 85

The following is a description of one example of the use of this invention: The ore of the Burro Mountain Company of New Mexico, United States of America (a 90 porphyry ore) when crushed gives a large proportion of interfering colloids and the method of treating the ore according to this invention corresponds very closely with that described with reference to the drawings in 95 the aforesaid United States Patent No. 1,102,874 and during the final grinding in the Hardinge mill there is added to the pulp a small proportion (say from  $\frac{1}{10}$  to  $\frac{1}{4}$  of a pound per ton of ore) of argol in addition to the modifying agent or oil already used. 100

Again, the ore of the Anaconda Copper Mine in Montana, United States of America when crushed produces slimes which 105 mainly pass through a 200 mesh screen and a large proportion of the slime is in a colloidal state. The ore has been experiment-

ally treated by the process described in the aforesaid United States Patent No. 1,102,874 and it is found that by agitating the modifying agents or frothing agents with a warm 5 solution of argol and then adding the mixture to a flotation circuit the result is greatly improved.

According to this invention the employment of a colloid agent such as tartaric acid 10 or argol in solution in the water or in the pulp may be combined with any of the known flotation processes.

Where sulfuric acid is employed in the flotation process, the colloid agent may be 15 introduced at an earlier stage than the sulfuric acid. For example the colloid agent may be used at the final grinding stage in the preparation of the pulp, or the colloid agent may be added to the pulp before the 20 flotation process begins, or the colloid agent and a modifying or frothing agent may be mixed or agitated with the pulp before the sulfuric acid is added. On the other hand the colloid agents of the type described can 25 be effectively employed in cases where sulfuric acid is not used.

Again, colloid agents of the type described may be used in the flotation process with or without the employment of oil and 30 with or without the employment of any other added agent.

What I claim as my invention and desire 35 to secure by Letters Patent is:—

1. A process for concentrating ores which 40 consists in mixing a powdered ore with water containing in solution a substance containing an acid radical of an oxyacid of the aliphatic group, containing also a small quantity of a mineral-frothing agent, agitating the mixture to form a froth and separating the froth.

2. A process for concentrating ores which

consists in mixing a powdered ore with water containing in solution argol, and containing also a small quantity of a mineral-frothing agent, agitating the mixture to 45 form a froth and separating the froth.

3. A process for separating certain constituents from an ore pulp containing colloidal slimes which consist in dissolving in 50 the pulp of such an ore a substance containing an acid radical of an oxyacid of the aliphatic group, adding to the pulp a small quantity of a mineral-frothing agent, agitating the mixture to form a froth, and separating 55 the froth.

4. A process for separating certain constituents from an ore pulp containing colloidal slimes which consists in dissolving argol in the pulp of such an ore, adding to 60 the pulp a small quantity of a mineral-frothing agent, agitating the mixture to form a froth, and separating the froth.

5. A process for concentrating ores which 65 consists in grinding the ore with water containing in solution a substance containing an acid radical of an oxyacid of the aliphatic group and containing also an air emulsifying agent, and then agitating the pulp to form a froth, and separating the froth.

6. A process for concentrating ores which 70 consists in grinding the ore with water containing argol in solution and containing also an air-emulsifying agent, and then agitating the pulp to form a froth, and separating 75 the froth.

In testimony whereof I have signed my name to this specification in the presence of two subscribing witnesses.

GEORGE ALBERT CHAPMAN.

Witnesses:

HENRY D. WILLIAMS,  
HARRY C. LEWIS.